

June 17, 1941.

R. BEATTIE

2,245,640

METHOD OF MOLDING PARAFFIN WAX

Filed April 10, 1936

Fig. 2.



Fig. 1.



Robert Beattie INVENTOR

BY

Robert D. Spurlock ATTORNEY

## UNITED STATES PATENT OFFICE

2,245,640

## METHOD OF MOLDING PARAFFIN WAX

Robert Beattie, Plainfield, N. J., assignor, by  
mesne assignments, of three-fourths to Tide  
Water Associated Oil Company, New York,  
N. Y., a corporation of Delaware

Application April 10, 1936, Serial No. 73,604

6 Claims.

(Cl. 18—55)

This invention relates to the forming of wax into bodies of defined shape. In its broader and more general aspects, the invention is concerned with the formation of shaped wax bodies (such as bars, cakes, and the like) by a continuous process enabling flexible control of production and economical manufacture. More particularly, the invention provides an improved method of forming solid shaped bodies of paraffin wax by an extrusion operation.

The present invention, while generally applicable to the formation of wax bodies or articles of various shapes and for various purposes, has particular utility in the refinery production of paraffin wax in cake form for shipment to industrial consumers. Paraffin wax production is an important adjunct of the petroleum industry, and, since the major industrial and commercial requirements are for refined wax of relatively high melting point (say, from 120° F. to 135° F. or even higher), it has long been the practice to form such wax into cakes or bars of standard size to facilitate packing, shipping, storing and handling this product.

This expedient is quite feasible because of the relatively high melting points of the waxes in question, there being little or no tendency for the cakes to soften and deform unduly under climatic conditions ordinarily encountered. As a convenience for industrial consumers, the use or handling of wax in cake form has, in fact, proved so satisfactory that cake forming has become, of necessity, a usual and required final step in the production of paraffin wax at the refinery. To this end, the refined wax is stored according to grade (i. e., melting point) in tanks from which it is fed, as required, in molten condition to a plurality of water-cooled molds in which the molten wax cools and hardens to form cakes, ordinarily conforming to a standard weight of eleven (11) pounds, and measuring 18 to 19 inches in length, 12 inches in width, and 1½ inches thick.

The formation of wax or bars by a simple casting operation in this manner is universal in the trade and has so been for a considerable number of years. Paraffin wax is a material of definitely crystalline nature and, therefore, is inherently well adapted to be formed into cakes or other defined shape by a casting operation. There are, however, certain fundamental defects in this traditional method of cake forming which interfere seriously with the efficiency and economy of the operation. The casting method with a slow cooling material such as wax, necessarily im-

poses batch operation with its attendant difficulties and drawbacks in the form of the unduly large number of units which must be maintained to meet varying market demands, the high initial investment which this implies, the excessive space and time requirements, especially for non-productive portions of the operation such as set-up and cleaning periods, and the like. These and other factors, both major and minor, have long commanded the attention of those skilled in the art, and many efforts have been made to find ways and means of improving the process but without material success. The desirability of providing a new method of wax cake forming, which will be free of many of the defects now encountered, is evident.

According to the present invention, the foregoing difficulties are obviated by the discovery that the formation of shaped wax bodies may be effected in an extrusion operation, and by the development therefrom of a novel process of wax body forming. As will appear more fully hereinafter, the invention thus attains by this discovery, and the improved process based thereon, desirable objects and advantages arising from continuous operation, flexible production control, operating economy, and low initial investment for equipment as compared with the older method.

In the accompanying drawings there is shown, for purposes of illustration, apparatus adapted for use in facilitating the operation of the process of the invention.

In the drawing, in which like reference characters denote like parts—

Figure I depicts, in generally diagrammatic form, an arrangement of apparatus adapted for wax body forming in accordance with present invention; and

Figure II depicts, in diagrammatic layout, an alternative embodiment which the extrusion apparatus of Figure I conveniently may take in practice.

The wax body forming process of the present invention may be regarded generally as comprising the main steps of (a) preparing a quantity or mass of unformed refined wax for body forming treatment; (b) extruding such wax supply continuously through a suitable die structure to form an extended continuous strip of uniform pre-determined cross-section; (c) continuously conditioning such strip as received through and from the die structure to avoid deformation; (d) severing the same transversely at spaced pre-determined intervals along the length thereof to form individual unitary wax bodies comprising

the desired wax cake product; and continuously maintaining such correlation of operating conditions, for example, temperature of the wax feed and operating temperatures maintained in the extrusion stage, with respect to the physical characteristics of wax under treatment, as to ensure continuity of operation and quality of product. The process further may include such secondary and supporting steps and refinements as pre-treatment of the wax supply to condition the same for the extrusion operation, two-stage extrusion, and intermediate de-aeration of the wax in process as by the inclusion of an intermediate vacuum conditioning step in the general process.

It has been determined that the successful adaptation of the principle of extrusion to the formation of wax bodies of defined shape necessitates (possibly because of the essentially crystalline nature of the material) a careful observance of temperature conditions at the several stages of the forming process as herein disclosed. Neglect of this factor apparently is fatal to the successful operation of the method and to the production of a satisfactory wax cake product. The precise optimum temperatures to be maintained in the wax feed supply and during the forming operation may, for purposes of practicability, be determined as a relatively narrow range, but undue deviation from the limits of such temperature range should be avoided.

It has been found, in semi-plant scale operation with waxes of different melting point, as, for example, 120° F., 125° F., 130° F., and 135° F., that the feed and the operating temperatures or temperature ranges vary for different grades of wax. Consequently, it is important to maintain a certain correlation between the physical properties of a given grade of wax, as evidenced most feasibly by its melting point, and the temperature conditions maintained in the several stages of the process.

Exploratory operation of the process under widely varying conditions has demonstrated that, as the feed wax enters the body forming means provided, its temperature should be sufficiently high to ensure complete merging of the several wax particles or crystal agglomerates into a substantially homogeneous mass during the body forming operation. At the same time, it is necessary to avoid a temperature approaching the melting point of the wax in process so closely as to interfere with continuous and substantially uniform feed to and through the extrusion unit, and with the formation of a firm undeformed wax body. Thus, the initial operating control in the process of the invention is concerned with the temperature maintained in the wax feed supply as it is delivered to the body forming operation. This is a unitary control in that, for a wax supply of given melting point, the same pre-determined feed temperature or temperature range should be maintained—and for different wax supplies of different grades or melting points, other feed temperatures or temperature ranges obtain in accordance with the prescribed melting point—feed temperature correlation. In the practice of the invention, this initial control has been found to be essential to successful operation.

In the body forming or extrusion operation of the process, the necessary operating control likewise relates to temperature; and may be regarded as a multiple control, as compared with the unitary nature of the initial or wax feed temperature control, in that the required temperature conditions for a given grade or melting point wax vary

in different stages of the body forming operation. That is to say, during the first stage of the body forming or extrusion operation certain temperature conditions should prevail, at another subsequent stage different temperature conditions are called for, and at the final stage as the formed body is emitted still other temperature conditions are maintained.

The operating control in the body forming or extrusion operation is of importance to proper operation and to production of a satisfactory wax cake product. As indicated, this control is multiple in nature as compared with the unitary character of the initial or feed supply temperature control. It differs further, in that the initial control is concerned with the average temperature throughout the body or mass of the wax feed; while the secondary or multiple control is concerned with the temperature of the outer layer or surface of the wax mass passing through the body forming operation.

The desirability of so controlling the temperature of the wax feeding to the body forming operation of the process naturally influences to some extent the form in which the wax feed is most advantageously supplied for the extrusion treatment. The wax feed may, of course, be supplied in a variety of ways as, for example, in the form of lumps, pieces, bars, masses, and the like, whether or not uniformly sized. It has been found quite convenient, however, to supply the wax feed in relatively comminuted form, as in small flakes or chips, which has the important advantage of facilitating the establishing and maintaining of the wax feed temperature within the required range. This method of preparing the wax feed likewise adds further flexibility to the process as a whole, since changes in the wax feed temperature in accordance with changes in the grades of wax being processed are more readily effected than might otherwise be the case.

If desired, a conventional type of wax flaking or chipping apparatus, generally available in most refineries, may be utilized for preparing the wax supply in the desired form for cake forming treatment. As ordinarily arranged and operated, this apparatus comprises a large cylindrical drum so disposed above a shallow pan or tray containing molten wax that the lower portion of the drum is continually submerged in the bath of melted wax. The surface of the drum is maintained at desired low temperatures, as by cooling water supplied internally thereto, and, as it rotates continuously, a thin film or coating of wax is picked up and hardens on the exposed areas of the outer drum surface. At a suitable point in the rotation of the drum this film or coating comes in contact with a shearing blade disposed parallel to the axis of the drum and in such relation to the surface thereof that, during the continued rotation of the drum, a wax coating is continuously and completely scraped off to fall in chip or flake form to a suitable receiver.

It will be understood, of course, that such other arrangements for preparing the wax supply in chip or flake form as may suggest themselves may be used, and further, that the wax feed may be in a form other than that of chips or flakes, without departing either from the scope or spirit of the invention.

Referring now more particularly to the accompanying drawings, Figure I depicts, in somewhat diagrammatic form, one cooperative assembly of units conventionally adaptable for use in carrying out the process of the present invention. Herein,

a wax flaker of substantial conventional design, generally designated at 10, is disposed in elevated relation to an extrusion unit 11, arranged to receive wax chips or flakes under gravity feed through a chute 12 from the flaker 10.

As shown, the wax flaker 10 includes the usual drum 13, wax pan 14, and scraper blade 15, but it has been found convenient, in the practice of the present invention, to modify slightly the customary relation of certain of the parts. Thus, it will be noted that the drum 13 is so positioned above the pan 14 that the lowermost portion of the drum surface is spaced somewhat from the level of the molten wax. With this arrangement, an air spray line 16 is provided, beneath the level of the wax in the pan and running lengthwise of the drum 13, which serves to transfer the molten wax in regulable quantity from the pan 14 to the cooled surface of the drum 13. The pan 14 likewise may be provided with steam coils 17 for maintaining the wax in the desired molten state. This modification of the conventional wax flaker set-up thus enables accurate regulation and control of such factors as amount of wax fed per unit of time, temperature of wax so fed, and occluded air content of the resulting flakes or chips as delivered from the flaker to the extrusion unit 11.

The wax flaker unit 10 may, of course, be utilized with its customary arrangement of parts as previously outlined and as generally familiar in the art; but in such instances there may be encountered the disadvantage of having available a relatively smaller degree of control over the rate at which the wax is supplied to the surface of the drum 13 from the pan 14. This defect may be overcome to some extent by employing the conventional flaker assembly together with an air spray line as hereinbefore described. In any event, it is to be clearly understood that there is contemplated a reasonable freedom of choice in regard to this step in the integrated operation of the invention.

The extrusion unit 11 comprises generally a cylindrical barrel 18 defining a laterally closed path of travel for the wax feed which passes therethrough under pressure as from a screw 19 rotatably disposed within the said barrel. At its discharge end, the barrel 18 is provided with a pre-forming section 20, having tapering upper and lower walls, presenting successive rectangular cross-sections of constant width and diminishing in area to that of the die orifice proper which accords with the transverse sectional dimensions of the cake to be formed. This section 20 functions to translate the combined rotary and forward motion of the wax feed through the barrel 18 into substantially linear forward motion into and through a die section 21 abutting the restricted end of the pre-forming section 20.

The extended continuous strip of wax issuing from the die 21 herein is received upon a series of rollers 22 arranged to support such strip without deformation in its continued travel away from the extrusion unit 11 to subsequent operations where it may be conditioned, severed, wrapped and packed.

As shown, the extrusion unit 11 is jacketed at suitable and desired sections thereof to enable temperature regulation and control at the several stages of the forming operation. Herein, a jacket 23 of substantial length is disposed around the barrel 18 intermediate its length; while a jacket 25 quite short in longitudinal extent is disposed around the tip or discharge end of the die section 21. An intermediate jacket 24 is so dis-

posed as to surround the forward portion of the pre-forming section 20 and the rearward or receiving end portion of the die section 21. The said jackets 23, 24, and 25 are adapted to receive 5 heat transmitting fluid, as for example, water or steam, or both, from any convenient sources (not shown) and may be equipped with thermocouples 26, or other desired temperature indicating devices to facilitate maintenance of necessary temperature conditions at the respective jacket sections of the walls of the unit 11.

Disposed above the rollers 22 are a plurality of sprays 27 through which cooling water from a manifold 28 is discharged upon the surface of the extruding wax strip or ribbon in order to set firmly the outer surface shell thereof. The said strip, after passing under the cooling water sprays 27, may be subjected to air drying as by upper and lower air jets 29 arranged above and below 15 the path of travel. Further drying of the formed wax body may be effected, if desired, by passing the same between felt pads 30 and 31, arranged to press lightly upon the upper and lower surfaces of the moving strip or ribbon, and disposed within 20 the path of travel. Further drying of the formed wax body may be effected, if desired, by passing the same between felt pads 30 and 31, arranged to press lightly upon the upper and lower surfaces of the moving strip or ribbon, and disposed within 25 a vacuum drying box 32.

In operation, with the aid of the apparatus depicted in Figure I and described as to its several cooperating units in the foregoing paragraphs, a supply of wax, say 130° F. melting point, is maintained in molten condition in the tray or pan 14 of the wax flaker unit 10, the steam coils 17 permitting control of the fluidity and temperature of the melted wax. This wax then is transferred at desired rates to the cooled outer surface of the drum 13 by means of the air spray line 16. The continuous rotation of the drum 13, by any convenient source of power, cooperating with the scraper blade 15 causes a supply of wax chips or flakes to be delivered through the chute 12 from the flaker 10 to the extrusion unit 11.

When operating upon 130° F. melting point wax, according to the instant body forming process, it has been found desirable to establish and maintain the supply of wax to the extrusion unit 45 within a temperature range of from 85° F. to 95° F. in order to obtain effective body forming operation for the production of a smooth compact cake product free of deformation and satisfactory in appearance. With this, as well as other 50 grades of wax, the molten wax supply to and in the flaker pan conveniently may be maintained at a temperature approximately 5° F. to 10° F. above the melting point of the wax in question; and the desired wax chip feed temperature obtained by regulation and control of the quantity 55 of molten wax supplied to the flaker drum, the temperature of the cooling water therewithin, and the amount and temperature of the air spray through the line 16.

As a precautionary measure, when using a wax flaker unit as described for the purpose of preparing the wax feed supply, the adjustment of the scraper blade 15 relative to the adjacent surface of the drum 13 should be checked occasionally to ensure the complete removal of the hardened wax coating continuously formed thereon. Otherwise, a thin permanent coating of wax may build up on the outer surface of the drum and, by its insulating effect, interfere with the desired rate of cooling the molten wax continuously transferred to the said surface from the pan 14.

As the wax feed passes into the receiving end of the extrusion barrel 18 it is pressed forward 70 under pressure by the screw 19. To ensure both

uniform forward travel and continuous merging of the wax particles, it is necessary to maintain a substantial co-efficient of friction between the inner surface of the barrel 18 and the wax carried by the screw 19. Consequently, cooling water is passed continuously through the jacket 23, and it has been determined that satisfactory operation results when this cooling water is maintained at a temperature of from 45° F. to 55° F. both for wax of 130° F. melting point and for other grades both higher and lower in melting point. The temperature of the cooling water flowing through the jacket 23 may be quite some lower in temperature than 45° F., but temperatures greatly in excess of 55° F. are to be avoided.

When the wax feed finally passes from the barrel 18, through the pre-forming section 20, into the section 21, it is beneficial to maintain the side walls of the unit at progressively higher temperatures than the walls of the barrel 18. Here, the co-efficient of friction between the wax and the inner walls of the die should be relatively low in order to provide for smooth passage of the wax body therethrough with gradually diminishing resistance in order to maintain substantially uniform linear forward velocity throughout the body of the wax. Hence, it has been found advantageous to maintain a fluid temperature in the jacket 24 of the order 90° F. to 100° F. while that in the final jacket 25 advantageously may be held at or somewhat above the melting point of the wax being processed.

In this illustrative operation, the body forming method of the invention was so conducted as to produce an extruded wax strip at the rate of approximately 40 linear inches per minute, the formed body or strip having a width of approximately 12 inches and a thickness of approximately 1½ inches.

The continuous body or strip of formed wax extruding from the die section 21 is, as before explained, conveniently received upon rollers 22; and, during its passage thereover, cooling water is sprayed upon the surface of the wax body to immediately cool and set the same to retain the smooth even surface imparted thereto by the final action of the die 21 and cooperating jacket 25. Following this treatment the extended body of wax may be air blown and passed between the absorbing surfaces of the vacuumized felt layers or pads 30 and 31 for drying. The wax strip then is ready for severing at spaced intervals into cakes of uniform length which may subsequently be wrapped, packaged, and stored in any desired manner.

As before indicated, it is important to the satisfactory production of wax cakes by the present process that the temperature of the wax as fed to the body forming or extrusion operation be established and maintained within a pre-determined range suitably correlated to the melting point of the wax being processed. In the foregoing description of the process in connection with the processing of 130° F. melting point wax, a temperature range of from 85° F. to 95° F. was shown to be a suitable one within which to maintain the temperature of the wax chips as fed to the extrusion unit. In other words, when forming shaped wax bodies from 130° F. melting point wax, the temperature of the wax chip feed should be established and maintained at not substantially less than 35° F. nor substantially more than 45° F. below the melting point of this particular grade of wax. Under the prescribed correlation of operating conditions to wax character-

istics, a continuous, uniformly sized strip was obtained which, upon severing at uniformly spaced intervals along the length thereof, produced cakes comparing very favorably in quality with those produced in the conventional casting operation as ordinarily employed in the art.

It is not possible to set forth an exact mathematical formula for calculating, for a given grade of wax, the precise differential to be established and maintained between the operating temperature of the wax feed and the melting point of the particular wax in question. Thus, as afore-mentioned, for 130° F. melting point wax a temperature differential within the range of 35° to 45° F. has given satisfactory results in large scale operation, while with different grades of wax (i. e., higher or lower melting points), other temperature differentials obtain. In general, it has been observed that the lower melting point waxes are best processed under conditions such that a larger differential exists than is necessary for waxes of higher melting point. For example, satisfactory cakes were obtained when extruding 120° F. melting point wax under a differential of from 40° F. to 50° F. maintained between the chip feed temperature and the wax melting point. On the other hand, wax of 135° F. melting point was processed to good quality cake product with an operating temperature differential in range of 35° F. to 40° F.; while 125° F. melting point wax formed well in the instant operation under substantially the same temperature correlation as hereinbefore indicated for 130° F. melting point wax. In all cases, however, the principle of suitably correlating the wax feed temperature to the melting point of the wax being processed is effective and apparently necessary to operation of the method. With this principle established as an important operating factor, the adaptation of the invention to forming shaped wax bodies from waxes other than those particularly enumerated herein will be readily achieved by those skilled in the art to whom the teachings of this specification are made available.

As to the temperature conditions maintained, by means of the jacket 24, at the intermediate stage of the body forming operation, the necessary correlation involves both the melting point of the wax in process and the rate of passage through the body forming operation. At this intermediate stage, defined by the last portion of the pre-forming section 20 and the first portion of the die section 21, the operating temperature should be so correlated to the melting point of the wax and to the rate of forward motion as to approach a condition of maximum plasticity of the surface layer of wax adjacent the inner wall surface of the unit without causing melting of this wax surface or layer. Thus, for different grades or melting point waxes, the temperature of the fluid passing through the jacket 24 will be adjusted in relation both to the melting point of the wax and to its rate of forward movement.

In like manner, the temperature of the fluid passing through the final jacket 25, disposed at the discharge end of the die piece 21, will be determined in correlative relations both to the melting point of the wax in process and to the rate of wax body passage or discharge; and will be so adjusted as to induce an incipient fusion of the very outer surface of the formed wax body at the point of discharge without affecting the rigidity of the body itself. By this practice, the emergence of the formed wax body is rendered

smooth and unimpeded, thereby avoiding deformation or surface roughness.

The extruded wax bodies or cakes formed by the practice of the present invention are characterized by a structure which presents in cross-section a series of concentric laminations or strata. This structure apparently is responsible for the enhanced strength, both in longitudinal and in transverse section, which these cakes exhibit in comparative tests with conventional cakes of the same melting point wax produced by the customary moulding or casting method. The extruded cakes may be substantially the same in density as the moulded cakes, or may run somewhat lighter, depending upon the amount of occluded air that is permitted to be entrained with the wax chips during the body forming operation. The amount of air present in the extruded cakes likewise may affect the surface appearance thereof, and it is possible, by regulation of the air content, to obtain cakes presenting in varying degree a generally mottled effect as desired.

The surface appearance of the extruded cakes may be further controlled by maintaining a relatively high jacket temperature at the discharge end of the die section 21 of the extrusion unit 11. Thus, by passing high temperature fluid, as steam, through the jacket 25, the temperature of the inner wall of said section 21 may be maintained at somewhat above the melting point of the wax in process, causing a thin layer of wax at the outer surface of the formed body to melt, which, upon immediate chilling as it emerges onto the rollers 22 and beneath the cooling water sprays 27, produces a smooth snow-white surface appearance similar to that presented by the wax cakes formed in a molding or casting operation. Experimental operation has demonstrated that this effect can readily be produced by the indicated procedure without deleterious effect upon other desired characteristics of the extruded cake, such as enhanced strength, uniform cross-sectional dimension, and the like.

A further embodiment of the present invention may be carried out with an arrangement of apparatus such as that shown diagrammatically in Figure II of the accompanying drawing. In this embodiment, provision is made for conditioning the wax feed at an intermediate point in the extrusion stage of the process; and, when operated according to Figure II as hereinbelow described, the process might aptly be considered as involving a two-stage extrusion operation.

The wax feed supply in this embodiment, as in that described in connection with Figure I, may be initially prepared in chip or flake form; and Figure II therefore does not include the wax flaker unit 10, a duplicated showing of this portion of the apparatus being unnecessary to an understanding of the features of the invention now to be presented.

Referring now more particularly to Figure II, there is there shown a wax body forming unit comprising generally a conditioning section and a forming section, the latter being in all essential respects identical with the extrusion unit 11 of Figure I. The conditioning section, indicated generally at 33 provides, in effect, a first extrusion operation, and has a horizontally disposed cylindrical barrel or chamber 34, adapted to receive a wax feed supply, as in chip or flake form. Rotatably mounted within the chamber 34 is a screw 35, the shaft of which comprises a rearward extension of the shaft of screw 19 in unit 11 and by means of which the wax supply is

passed forwardly under pressure. At the discharge end of the barrel 34 there is fixed a perforated plate 36, through the openings in which the wax feed is forced or extruded to 5 emerge as a plurality of relatively small ribbons or pencil-like sections, thereby presenting at emergence a large exposed surface area relative to the total mass. The ribbons of wax thus extruded through the plate 36 are received in a 10 confined space or chamber 37 which is arranged to be evacuated by any convenient means indicated diagrammatically at 38. At the far end of the chamber 37 is attached an extrusion unit 11 similar in all respects to that shown in Figure I and 15 previously described in connection therewith. For convenience of assembly and operation, the extruding screws 35 and 19 respectively may be provided with a common shaft as shown, this an arrangement permitting the use of common drive mechanism (not shown) for the two extrusion units. The screw 35 operating in the first extrusion unit 33 is, of course, discontinued just before the perforated plate 36; while the screw 19 in the second extrusion unit 11 has its first turn spaced from 20 the opposite or discharge side of said plate. The wax, emerging in ribbon-like or pencil-like form through the plurality of openings in the perforated plate 36, thus passes through the evacuated chamber 37 and feeds directly to the unit 11, where it is subjected to the final body forming treatment hereinbefore set forth.

When practicing the invention with a form of apparatus such as that just described, a supply of wax chips or flakes passes from a flaker unit 10 by gravity through a chute 12 to the feed end of the barrel 34 of the preliminary extruder 33. Here, the wax chips are pressed forwardly by the continuous rotation of the screw 35 and forced or extruded through the perforated plate 36 into the evacuated chamber 37. As previously indicated, the wax emerging through the plate 36 in the form of a plurality of thin pencils or ribbons, presents a very large area of exposed surface relative to the mass; and thus is readily responsive to the de-aerating action of evacuating means 38 operatively associated with the chamber 37. Whatever means is selected to create the desired vacuum advantageously may include regulatory control for varying the degree of vacuum imposed upon the said chamber in order to enhance the flexibility of the operation, as, for example, to meet possible variations in the amount of occluded air carried by the wax, degree of de-aeration desired, variations in the wax feed rate, 45 and the like. It will be understood, of course, that the particular evacuating means selected forms no part of the present invention, and since many conventional and well-known devices are readily available, it is deemed unnecessary to include here any detailed showing or description of a specific illustrative device.

In operation with this embodiment of the invention, as with that first described, it will be understood that the prescribed operating controls and correlations must be observed.

I claim:

1. In a method of forming paraffin wax into bodies of defined shape by continuously extruding a supply of wax in relatively comminuted solidified state through suitably dimensioned body forming means, the improvement which comprises maintaining, during the body forming operation, a differential between the wax supply temperature and the melting point of the wax of not sub-

stantially more than fifty (50) nor substantially less than thirty (30) degrees Fahrenheit.

2. In a method of forming paraffin wax into bodies of defined shape by continuously extruding a supply of wax in relatively comminuted solidified state through suitably dimensioned body forming means, the improvement which comprises maintaining, during the body forming operation, a differential between the wax supply temperature and the melting point of the wax of not substantially more than fifty nor substantially less than thirty degrees Fahrenheit, the differential selected for any given melting point wax being of the higher order for lower melting point waxes and of the lower order for higher melting point waxes.

3. In a method of forming paraffin wax into bodies of defined shape, by continuously feeding a supply of wax in solidified state, maintained at a temperature substantially below the melting point thereof, to and through a relatively elongated chamber of restricted cross-section terminating in body forming and shape defining means operatively associated therewith, the improvement which comprises maintaining the walls of said chamber at a temperature below that of said wax supply passing therethrough, and maintaining said means at a temperature well above that of said chamber walls.

4. The method of forming paraffin wax into bodies of defined shape, which comprises continuously feeding a supply of wax in relatively comminuted solidified state, maintained at a temperature substantially below the melting point thereof but so correlated thereto that body forming conditions obtain during the body forming operation, to and through a relatively elongated chamber of restricted cross-section terminating in body forming and shape defining means operatively associated therewith, maintaining the walls of said chamber at a temperature within the range of forty-five to fifty-five degrees Fahrenheit, and maintaining successive zones in said means at successively increasing temperatures, the zone of

said means adjacent the point of emergence of said wax being at a temperature substantially that of the melting point of the wax passing therethrough.

5. The method of forming paraffin wax having a melting point not substantially less than 120° F., into bodies of defined shape, which comprises continuously feeding a supply of wax in relatively comminuted solidified state, maintained at a temperature which is at least 30° F. below the melting point of the wax treated, to and through a relatively elongated chamber of restricted cross-section terminating in body forming and shape defining means operatively associated therewith, maintaining the walls of said chamber at a temperature within the range of 45 to 55° F., and maintaining successive zones in said means at successively increasing temperatures, the zone of said means adjacent the point of emergence of said wax being at a temperature substantially that of the melting point of the wax passing therethrough.

6. The method of forming paraffin wax having a melting point not substantially less than 120° F., into bodies of defined shape, which comprises continuously feeding a supply of wax in relatively comminuted solidified state, maintained at a temperature which is at least 30° F. below the melting point of the wax treated, to and through a relatively elongated chamber of restricted cross-section terminating in body forming and shape defining means operatively associated therewith, maintaining the walls of said chamber at a temperature within the range of 45 to 55° F., and maintaining successive zones in said means at successively increasing temperatures, the zone of said means adjacent the point of emergence of said wax being at a temperature substantially that of the melting point of the wax passing therethrough, the zone intermediate said chamber and the point of emergence of said wax being maintained at a temperature within the range of 90 to 100° F.

ROBERT BEATTIE.